# EUROPEAN PATENT SPECIFICATION

(11) **EP 2 822 718 B1**
(45) Date of publication and mention of the grant of the patent: **07.08.2019**
(21) Application number: 13712412.9
(22) Date of filing: 08.03.2013
(51) Int. Cl.: B22F 3/115, B22F 5/02, B22F 9/08, C22C 33/02

(54) **THERMAL SPRAY APPLICATIONS USING IRON BASED ALLOY POWDER**
WÄRMESPRÜHANWENDUNGEN MIT EINEM EISENLEGIERUNGSPULVER
APPLICATIONS DE PROJECTION THERMIQUE UTILISANT UNE POUDRE D'ALLIAGE À BASE DE FER

(30) Priority: 09.03.2012 US 201261608853 P
(43) Date of publication of application: 14.01.2015
(73) Proprietor: Tenneco Inc., Lake Forest, IL 60045 (US)
(72) Inventor: CHRISTOPHERSON, JR., Denis, B., Waupun, WI 53963 (US); L'ESPERANCE, Gilles, Candiac, Quebec J5R6 (CA); KOTH, Jeremy, Sun Prairie, WI 53590 (US); BEAULIEU, Phillipe, Montréal H2R 2A4 (CA); FARTHING, Leslie John, Rugby CV22 5JW (GB); SCHOENWETTER, Todd, WI 53916 (US)
(74) Representative: HGF Limited
(86) International application number: PCT/US2013/029792
(87) International publication number: WO 2013/134606

(56) References cited:
- EP-A2- 0 266 149
- EP-A2- 0 266 149
- WO-A2-2009/126674
- WO-A2-2009/126674
- WO-A2-2009/126674
- CN-A- 102 286 702
- CN-A- 102 286 702
- US-B2- 6 887 585
- US-B2- 6 887 585
- US-B2- 7 998 238
- US-B2- 7 998 238
- US-B2- 7 998 238

## Description

### BACKGROUND OF THE INVENTION

### 1. Field of the Invention

This invention relates generally to wear resistant thermal spray powders, methods of forming the same, and applications thereof.

### 2. Related Art

Thermal spray techniques are used to apply wear resistant coatings to automotive engine components, such as pistons and piston rings. The coatings can protect the surface of the piston rings from wear as the piston slides along the cylinder. The coatings also reduce corrosion and oxidation of the piston caused by exposure to extreme temperatures and pollutants in the combustion chamber of the engine. Such wear resistant coatings have been formed from various ceramic materials, chromium-based powders, and molybdenum based powders. Examples of thermal spraying techniques include combustion, electrical discharge, cold spraying, and laser.

WO2009/126674 describes a pre-sintered powder metal composition with over 3.0 wt % carbon, about 13 wt % chromium, about 2.5 wt % tungsten, about 4 wt % vanadium, about 1.5 wt % molybdenum and an oxygen content less than about 0.5 wt %.
US 6887 585 B2 describes a wear-resistant coating for the bearing surfaces and flanks of piston rings, the wear-resistant coating comprising a mechanically alloyed powder mixture obtainable by mechanical alloying, said powder mixture including a metallic matrix comprising at least one of nickel land iron, and further comprising an iron-alloying element.
EP 0266149 A2 describes a method of producing a wear-resistant metal member comprising the steps of spraying an alloy onto a surface of a metal member in a reduced pressure atmosphere by plasma spraying to form a sprayed layer on said surface, said alloy consisting essentially of by weight, 2 to 10% C, 18 to 60% Cr, 0.3 to 20% V, 25% or less Mo, 25% or less W, 10% or less Hf and the balance being Fe in a proportion of 20% or greater. The sprayed layer is subjected to a hardening treatment, followed by quenching and then a tempering treatment.

### SUMMARY OF THE INVENTION

The present disclosure describes a method of forming a wear resistant component comprising the steps of: spraying a powder metal material, wherein the powder metal material consists of 3.0 to 7.0 wt. % carbon, 10.0 to 25.0 wt. % chromium, 1.0 to 5.0 wt. % tungsten, 3.5 to 7.0 wt. % vanadium, 1.0 to 5.0 wt. % molybdenum, not greater than 0.5 wt. % oxygen, the balance being iron and impurities, based on the total weight of the powder metal material.

The thermal spray powder provides exceptional wear resistance at a low cost relative to other materials used in thermal spray techniques. The thermal spray powder also has a lower melting point and therefore requires lower temperatures during the thermal spray technique, which conserves energy. The thermal spray powder may also be applied to a metal body, such as a piston or piston ring, without causing damage to the body. In addition, during the thermal spray technique, the thermal spray powder may provide improved oxidation resistance compared to other ferrous based materials used in thermal spray techniques.

### BRIEF DESCRIPTION OF THE DRAWINGS

Other advantages of the present invention will be readily appreciated, as the same becomes better understood by reference to the following detailed description when considered in connection with the accompanying drawings wherein:
Figure 1 illustrates a high velocity oxygen fuel spraying (HVOF) chamber gun spraying a thermal spray powder on an outer surface of a piston according to one embodiment of the invention;
Figure 2 illustrates the HVOF chamber gun spraying the thermal spray powder on an outer surface of a piston ring according to another embodiment of the invention;
Figure 3 is a cross-sectional view of the piston ring of Figure 2 along line 3;
Figure 4 illustrates the HVOF chamber gun spraying the thermal spray powder to form a spray-formed part according to another embodiment of the invention; and
Figure 5 is a schematic illustration of an exemplary process used to form the thermal spray powder.

### DETAILED DESCRIPTION

The powder metal material, also referred to as a thermal spray powder 20, is formed by atomizing a melted iron based alloy including carbon (C), chromium (Cr), tungsten (W), vanadium (V), molybdenum (Mo), and iron (Fe). The thermal spray powder 20 is iron-based and optionally includes other components, such as cobalt (Co), niobium (Nb), titanium (Ti), manganese (Mn), sulfur (S), silicon (Si), phosphorous (P), zirconium (Zr), and tantalum (Ta).

The thermal spray powder 20 includes chromium, tungsten, vanadium, and molybdenum in amounts sufficient to provide exceptional wear resistance at a reduced cost, compared to other thermal spray materials. These elements are also present in amounts sufficient to form metal carbides. In one embodiment, the thermal spray powder 20 includes 10.0 to 25.0 wt. % chromium, preferably 11.0 to 15.0 wt. % chromium, and most preferably 13.0 wt. % chromium; 1.0 to 5.0 wt. % tungsten, preferably 1.5 to 3.5 wt. % tungsten, and most preferably 2.5 wt. % tungsten; 3.5 to 7.0 wt. % vanadium, preferably 4.0 to 6.5 wt. % vanadium, and most preferably 6.0 wt. % vanadium; 1.0 to 5.0 wt. % molybdenum, preferably 1.0 to 3.0 wt. % molybdenum, and most preferably 1.5 wt. % molybdenum.

The thermal spray powder 20 includes the carbon in an amount sufficient to provide metal carbides in an amount greater than 15 vol. %, based on the total volume of the thermal spray powder 20. In one embodiment, the thermal spray powder 20 includes at least 3.0 wt. % carbon, or 3.0 to 7.0 wt. % carbon, and preferably about 3.8 wt. % carbon, based on the total weight of the thermal spray powder 20. As the amount of carbon in the thermal spray powder 20 increases so does the hardness of the thermal spray powder 20. This is because greater amounts of carbon form greater amounts of carbides during the atomization step, which increases the hardness. The amount of carbon in the thermal spray powder 20 is referred to as carbon total (Cₜₒₜ).

The thermal spray powder 20 also includes a stoichiometric amount of carbon (C_{stoich}), which represents the total carbon content that is tied up in the alloyed carbides at equilibrium. The type and composition of the carbides vary as a function of the carbon content and of the alloying elements content.

The C_{stoich} necessary to form the desired amount of metal carbides during atomization depends on the amount of carbide- forming elements present in the thermal spray powder 20. The C_{stoich} for a particular composition is obtained by multiplying the amount of each carbide-forming element by a multiplying factor specific to each element. For a particular carbide-forming element, the multiplying factor is equal to the amount of carbon required to precipitate 1 wt. % of that particular carbide-forming element. The multiplying factors vary based on the type of precipitates formed, the amount of carbon, and the amount of each of the alloying elements. The multiplying factor for a specific carbide will also vary with the amount of carbon and the amount of the alloying elements.

For example, to form precipitates of (Cr_{23.5}Fe_{7.3}V_{63.1}Mo_{3.2}W_{2.9})₈C₇, also referred to as M₈C₇, in a thermal spray powder 20, the multiplying factors of the carbide- forming elements are calculated as follows. First, the atomic ratio of the M₈C₇ carbide is determined: 1.88 atoms of Cr, 0.58 atoms of Fe, 5.05 atoms of V, 0.26 atoms of Mo, 0.23 atoms of W, and 7 atoms of C. Next, the mass of each element per one mole of the M₈C₇ carbide is determined: V = 257.15 grams, Cr = 97.76 grams, Fe = 32.62 grams, Mo = 24.56 grams, W = 42.65 grams, and C = 84.07 grams. The weight ratio of each carbide-forming element is then determined: V = 47.73 wt. %, Cr = 18.14 wt. %, Fe = 6.05 wt. %, Mo = 4.56 wt. %, W = 7.92 wt. %, and C = 15.60 wt. %. The weight ratio indicates 47.73 grams of V will react with 15.60 grams of C, which means 1 gram of V will react with 0.33 grams of C. To precipitate 1.0 wt. % V in the M₈C₇ carbide you need 0.33 wt. % carbon, and therefore the multiplying factor for V is 0.33. The same calculation is done to determine the multiplying factor for Cr = 0.29, Mo = 0.06, and W = 0.03.

The C_{stoich} in the thermal spray powder 20 is next determined by multiplying the amount of each carbide-forming element by the associated multiplying factor, and then adding each of those values together. For example, if the thermal spray powder 20 includes 4.0 wt. % V, 13.0 wt. % Cr, 1.5 wt. % Mo, and 2.5 wt. % W, then C_{stoich} = (4.0^{∗}0.33) + (13.0^{∗}0.29) + (1.5^{∗}0.06) + (2.5^{∗}0.03) - 5.26 wt. %.

In addition, the thermal spray powder 20 includes a Ctₒₜ/ C_{stoich} amount less than 1.1. Therefore, when the thermal spray powder 20 includes carbon at the upper limit of 7.0 wt. %, the C_{stoich} will be 6.36 wt. % carbon (7.0 wt. % carbon / 1.1).

The table below provides examples of other carbide types that can be found in the thermal spray powder 20, and multiplying factors for Cr, V, Mo, and W for generic carbide stoichiometry. However, the metal atoms in each of the carbides listed in the table could be partly replaced by other atoms, which would affect the multiplying factors.

| **Element** | **Carbide type** | **Example of stoichiometry** | **Multiplying factor f_{M} (w%/w%)** |
|---|---|---|---|
| Cr | M₇C₃ | Cr_{3.5}Fe_{3.5}C₃ | 0.20 |
| | | Cr₄Fe₃C₃ | 0.17 |
| | | (Cr₃₄Fe₆₆)₇C₃ | 0.29 |
| V | M₈C₇ | (V₆₃Fe₃₇)₈C₇ | 0.33 |
| Mo | M₆C | Mo₃Fe₃C | 0.04 |
| | | Mo₂Fe₄C | 0.06 |
| W | M₆C | W₃Fe₃C | 0.02 |
| | | W₂Fe₄C | 0.03 |

The metal carbides are formed during the atomization process and are present in an amount of at least 15.0 vol. %, but preferably in an amount of 40.0 to 60.0 vol. %, or 47.0 to 52.0 vol. %, and typically about 50.0 vol. %. In one embodiment, the thennal spray powder 20 includes chromium-rich carbides, molybdenum-rich carbides, tungsten-rich carbides and vanadium-rich carbides in a total amount of about 50.0 vol. %.

The metal carbides have a nanoscale microstructure. In one embodiment, the metal carbides have a diameter between 1 and 400 nanometers. The fine nano-carbide structure may improve the adherence of the thennal spray powder 20 to an outer surface 22, 122 of a metal body 24, 124. Therefore, a wear resistant coating formed of the thermal spray powder 20 is less prone to flaking, chipping, and delamination. The fine carbide structure may also provide a more homogeneous microstructure, and therefore an improved impact and fatigue resistance compared to thermal spray materials with coarser carbide microstructures. As alluded to above, the carbides can be of various types, including M₈C₇, M₇C₃, MC, M₆C, M₂₃C₆, and M₃C, wherein M is at least one metal atom, such as Fe, Cr, V, Mo, and/or W, and C is carbon. In one embodiment, the metal carbides are selected from the group consisting of: M₈C₇, M₇C₃, MC, M₆C, wherein MₐC₇ is (V₆₃Fe₃₇)₈C₇, M₇C₃ is selected from the group consisting of: (Cr₃₄Fe₆₆)₇C₃, Cr_{3 5}Fe₃. ₅C₃, and Cr₄Fe₃C₃; and M₆C is selected from the group consisting of: Mo₃Fe₃C, Mo2Fe4C, W₃Fe₃C, and W₂Fe₄C.

The microstructure of the thermal spray powder 20 also includes nanoscale austenite, and may include nanoscale martensite, along with the nanoscale carbides. The carbon is also present in an amount sufficient to limit oxidation of the thermal spray powder 20 during the thermal spray process. Oxidation can occur due to poor atmosphere control, lack of cleanliness, and temperature during the thermal spray process.

The remaining balance of the thermal spray powder 20 composition is iron. The thermal spray powder 20 typically has a microhardness of 800 to 1 ,500 Hv 50. The high hardness contributes to the exceptional wear resistance of the wear resistant coating 26 and the fine structure should improve toughness. The microhardness of the thermal spray powder 20 increases with increasing amounts of carbon.

In one exemplary embodiment, the thermal spray powder 20 includes 3.8 wt. % carbon, 13.0 wt. % chromium, 2.5 wt. % tungsten, 4.0-6.0 wt. % vanadium, 1.5 wt. % molybdenum, 0.2 wt. % oxygen, impurities in an amount not greater than 2.0 wt. % and the balance being iron, based on the total weight of said thermal-sprayed powder metal material.

The thermal spray powder 20 of the exemplary embodiment has a melting point of about 1,235° C (2,255° F), and it will be completely melted at that temperature. The melting point of thermal spray powder 20 will however vary slightly as a function of the carbon content and alloying element content. However, the thermal spray powder 20 may include a small fraction of a liquid phase at a temperature as low as 1 ,150° C. The low melting point provides several advantages during the thermal spray process, compared to thermal spray materials having higher melting points. Less energy is needed to apply the thermal spray powder 20 to the outer surface 22 of the body 24 being coated. The thermal spray powder 22 can be sprayed at a lower temperature, which may provide less heat input to the body 24 being coated, less manufacturing equipment wear, possibly lower porosity in the wear resistant coating 26, and less oxidation of the thermal spray powder 20 during the spraying process. The lower melting point also provides the opportunity to use a cold spraying technique.

The thermal spray powder 20 is formed by water or gas atomizing a melted iron based alloy. An exemplary process of forming the thermal spray powder 20 using water atomization is shown in Figure 5. However, the water atomization step could be replaced by a gas atomization step. In one embodiment, the iron based alloy provided prior to atomization includes 3.0 to 7.0 wt. % carbon, 10.0 to 25.0 wt. % chromium, 1.0 to 5.0 wt. % tungsten, 3.5 to 7.0 wt. % vanadium, 1.0 to 5.0 wt. % molybdenum, and at least 40.0 wt. % iron. The iron based alloy is typically provided as a pre-alloy including the carbon, chromium, tungsten, vanadium, molybdenum, and iron. The iron based alloy also has a low oxygen content, preferably not greater than 0.5 wt. %. The carbon content of the iron based alloy is sufficient to protect the alloy from oxidizing during the melting and atomizing steps.

Once the iron based alloy is melted, it is fed to a water atomizer or a gas atomizer. The high carbon content of the iron based alloy decreases the solubility of the oxygen in the melted iron based alloy. Depleting the oxygen level in the melted iron based alloy has the benefit of shielding the carbide-forming elements from oxidizing during the melting and atomizing steps. The relatively high carbon content allows the austenite, or possibly martensite, to form in the matrix of the thermal spray powder 20, in which the carbides precipitate, during the atomizing step. Increasing the amount of carbide-forming alloying elements in the iron based alloy can also increase the amount of carbides formed in the matrix during the atomizing step.

In the atomizer, a stream of the melted iron based alloy is impacted by a flow of high-pressure water or gas which disperses and rapidly solidifies the melted iron based alloy stream into fully alloyed metal droplets. Gas atomization typically yields particles having a round shape, whereas water atomization typically yields particles of irregular shape. Preferably, each droplet possesses the fully alloyed chemical composition of the melted batch of metal, including at least 3.0 wt. % carbon, 10.0 to 25.0 wt. % chromium, 1.0 to 5.0 wt. % tungsten, 3.5 to 7.0 wt. % vanadium, 1.0 to 5.0 wt. % molybdenum, and at least 40.0 wt. % iron. Each droplet also preferably includes a uniform distribution of carbides. The main elements of the droplets are protected from oxidation by the high carbon content of the powder during the melting and atomizing steps. The high carbon content and low oxygen content also limits the oxidization during the atomizing step. However, the outside surface of the droplets may become oxidized, possibly due to exposure to water or unprotected atmosphere. Some properties can be improved using gas atomization over water atomization, for example better flow, apparent density, and lower oxygen content.

The atomized droplets are then passed through a dryer and into a grinder where the atomized material is mechanically ground or crushed, and then sieved. The hard and very fine nano-structure of the droplets improves the ease of grinding. A ball mill or other mechanical size reducing device may be employed. In addition, the droplets could be annealed prior to grinding the droplets, but no annealing step is required prior to grinding the droplets, and typically no annealing step is conducted. If an outer oxide skin is formed on the atomized droplets during the atomization step, the mechanical grinding fractures and separates the outer oxide skin from the bulk of the droplets. The ground droplets are then separated from the oxide skin to yield the atomized thermal spray powder 20 and oxide particles 30, as shown in Figure 5. In certain cases, such as when gas atomization is used, the outer oxide skin is minimal and can be tolerated without removal. However, the mechanical grinding step can still be used to fracture and reduce the size of the droplets. The thermal spray powder 20 may be further sorted for size, shape and other characteristics normally associated with powder metal. The thermal spray powder 20 can then be used to form a wear resistant component 28, 128, 228 such as a piston or piston ring.

Figure 1 illustrates an example of the wear resistant component 28 including the thermal spray powder 20. In Figure 1, the wear resistant component 28 is a piston including a body 24, specifically a skirt, presenting an outer surface 22. The thermal spray powder 20 is applied to the outer surface 22 of the body 24 by a thermal spraying technique to form a wear resistant coating on the outer surface 22. The wear resistant coating typically has a microhardness of 800 to 1 ,500 Hv₅ₒ. Figure 2 illustrates another example of the wear resistant component 128 including the thermal spray powder 20. The wear resistant component 128 includes a body 124, specifically an uncoated piston ring, presenting an inner surface 136 surrounding a center axis A and an outer surface 122 facing opposite the inner surface 136. The thermal spray powder 20 is applied to the outer surface 122 by a thermal spraying technique to form a wear resistant coating on the outer surface 122.

The thermal spray powder 20 can also be used to form wear resistant coatings on other components (not shown), for example turbine blades, transmission parts, exhaust system components, crankshafts, other automotive components, pulp and paper rollers, oil and petrochemical drilling components, golf clubs, and surgical applications.

Figure 4 is another example of the wear resistant component 228, specifically a piston ring, wherein the wear resistant component 228 consists entirely of the thermal spray powder 20. The wear resistant component 228 presents an inner surface 236 surrounding a center axis A and an outer surface 222 facing opposite the inner surface 236. This wear resistant component 228 is referred to as a spray-formed part. The spray-formed part typically has a microhardness of 800 to 1 ,500 Hv₅ₒ.

Various thermal spray techniques can be used to form the wear resistant component 28, 128, 228. Four typical thermal spray techniques are combustion, electrical discharge, cold spray, and laser. Each thermal spray technique includes spraying the thermal spray powder 20, either onto the outer surface 22, 122 of the body 24, 124 to form the wear resistant coating, or onto a substrate 238 to form the spray-formed part. The spraying step includes accelerating the thermal spray powder 20 at a high velocity, which can be up to a supersonic velocity. Once the thermal spray powder 20 has been sprayed at the high velocity to form the coating or the spray-formed part, it can be referred to as a thermal- sprayed powder or thermal-sprayed coating. The combustion, electrical discharge, and laser techniques include melting the thermal spray powder 20 before spraying the melted powder. These techniques include heating the thermal spray powder 20 and then accelerating the heated thermal spray powder 20 to the outer surface 22, 122 of the body 24, 124 or onto the substrate 238, at a high velocity while the thermal spray powder 20 is heated.

One example of the combustion technique includes flame spraying, such as powder flame spraying or wire flame spraying. Another example of the combustion technique is high velocity oxygen fuel spraying (HVOF), which involves oxygen and gaseous fuels (HVOF-G) or liquid fuels (HVOF-K).

The electrical discharge technique can include plasma spraying or wire arc spraying. The plasma spraying is typically conducted under inert gas (IPS), a vacuum (VPS), or by dispersing the thermal spray powder 20 in a liquid suspension before injecting the thermal spray powder into a plasma jet (SPS). The plasma spraying can also include atmospherical plasma spraying (APS), high pressure plasma spraying (HPPS), water-stabilized plasma spraying (WSPS), reactive plasma spraying (RPS), or underwater plasma spraying (UPS). If nitrogen is used as the inert gas during the plasma spraying process, there is a potential to form vanadium carbonitrides, thus improving hardness and wear resistance. This potential is controlled by the processing parameters and the chemistry of the thermal spray powder 20 before the spraying process.

The most preferred thermal spray techniques are powder flame spraying, plasma spraying, cold spraying, and high velocity oxygen fuel spraying (HVOF). Figures 1, 2, and 4 illustrate a step in the HVOF process, wherein a HVOF chamber gun sprays the thermal spray powder 20 on the outer surface 22, 122 of the body 24, 124, or onto the substrate 238. The HVOF chamber gun includes a pressurized combustion chamber 32 in fluid communication with a nozzle 34. The combustion chamber 32 contains a mixture of carrier gas, such as oxygen, and fuel, such as of acetylene, hydrogen, propane, or propylene. The mixture is ignited to produce a high-pressure flame and creating a pressure in the combustion chamber. The flame is formed through the nozzle 34 to accelerate the earner gas to a high velocity, which can be up to a supersonic velocity. The thermal spray powder 20 is then fed axially into the high pressure combustion chamber 32 or directly through the side of the nozzle 34. The carrier gas accelerates the thermal spray powder 20 out of the HVOF chamber gun at a high velocity.

In the embodiments of Figures 1 and 2, the thermal spray powder 20 is applied to the outer surface 22, 122 of the body 24, 124 to form the wear resistant coating. Figure 3 shows a thickness t of the wear resistant coating applied to the body 124 of Figure 2. The thickness depends on the thermal spray technique used, design of the body 124, and application of the wear resistant component 28. In one embodiment, the thickness of the wear resistant coating is 20 to 200 microns.

The method of forming the wear resistant component 28 can optionally include a post-spraying heat treatment. In one embodiment, the method includes annealing the thermal spray powder 20 after it is applied to the body 24, 124 or formed into the spray-formed part. The annealing or other heat treatment step could modify the micro structure of the thermal spray powder 20 by making it coarser. For example, the metal carbides could have diameter of at least one micron, rather than between 1 and 400 nanometers.

Another aspect of the invention provides a method of forming the wear resistant component 228, wherein the wear resistant component 228 is a spray-formed part consisting of the thermal spray powder 20, such as the piston ring of Figure 4. The spray- formed part is manufactured by spraying the thermal spray powder 20 onto the substrate 238 to a thickness of up to 500 millimeters. The spray-forming process is a near-net-shape process and includes capturing a spray of powder on a moving substrate, as described in the ASM Handbook, Volume 7. This process provides several advantages, including densities greater than 98%, fine equiaxed grains, no macroscopic segregation, absence of prior particle boundaries, enhanced mechanical properties, material/ alloying flexibility, and a high rate of deposition, such as greater than 2 kg/second.

In addition, the thermal spray powder 20 could be co-sprayed with other powders to form the wear resistant component 28, 128, 228, either the resistant coating or the spray-formed part. Examples of other powders that could be co-sprayed with the thermal spray powder 20 of the present invention include intermetallics, other hard phases, and metallic alloys. The wear resistant coatings 26 and spray-formed parts including the co- sprayed powders could provide a wide range of microstructures, different from the microstructures provided by the thermal spray powder 20 alone.

Obviously, many modifications and variations of the present invention are possible in light of the above teachings and may be practiced otherwise than as specifically described while within the scope of the claims.

## Claims

1. A method of forming a wear resistant component, comprising the steps of: thermal spraying a powder metal material, wherein the powder metal material consists of 3.0 to 7.0 wt. % carbon, 10.0 to 25.0 wt. % chromium, 1.0 to 5.0 wt. % tungsten, 3.5 to 7.0 wt. % vanadium, 1.0 to 5.0 wt. % molybdenum, not greater than 0.5 wt. % oxygen, and the balance being iron and impurities, based on the total weight of the powder metal composition.

2. A method according to claim 1 wherein the thermal spraying step is a thermal spray technique selected from the group consisting of: powder flame spraying, plasma spraying, cold spraying, and high velocity oxygen fuel spraying (HVOF).

3. A method according to claim 1 wherein the thermal spray technique includes providing a combustion chamber containing a mixture of fuel and oxygen; igniting the mixture of fuel and oxygen; and feeding the powder metal material into the combustion chamber after the igniting step to accelerate the powder metal material.

4. A method according to claim 3 wherein the igniting step includes creating a pressure in the combustion chamber, and accelerating the powder metal material up to a supersonic velocity.

5. A method according to claim 1 including providing a body, and wherein the spraying step includes spraying the powder metal material onto the body.

6. A method according to claim 1 wherein the spraying step forms the wear resistant component, and the wear resistant component is a piston ring presenting an inner surface surrounding a center axis and an outer surface facing opposite the inner surface.

7. A method according to claim 1 including forming the powder metal material by the steps of:
providing a melted iron based alloy including 3.0 to 7.0 wt. % carbon, 10.0 to 25.0 wt. % chromium, 1.0 to 5.0 wt. % tungsten, 3.5 to 7.0 wt. % vanadium, 1.0 to 5.0 wt. % molybdenum, not greater than 0.5 wt. % oxygen, and at least 40.0 wt. % iron, based on the total weight of the melted iron based alloy;
atomizing the melted iron based alloy to provide atomized droplets of the iron based alloy; and
grinding the atomized droplets.

8. A method according to claim 7, wherein the atomizing step includes forming metal carbides in the iron based alloy in an amount of at least 15.0 vol. %, based on the total volume of the iron based alloy.

9. A method according to claim 8, wherein the metal carbides are selected from the group consisting of: M8C7, M7C3, M6C, wherein M is at least one metal atom and C is carbon.

10. A method according to claim 9, wherein M8C7 is (V63Fe37)8C7; M7C3 is selected from the group consisting of: (Cr34Fe66)7C3, Cr3.5Fe3.5C3, and Cr4Fe3C3; and M6C is selected from the group consisting of: Mo3Fe3C, Mo2Fe4C, W3Fe3C, and W2Fe4C.

11. A method according to claim 1, wherein the powder metal material consists of: 3.8 wt. % carbon, 13.0 wt. % chromium, 2.5 wt. % tungsten, 6.0 wt. % vanadium, 1.5 wt. % molybdenum, 0.2 wt. % oxygen, impurities in an amount not greater than 2.0 wt. % and the balance being iron, based on the total weight of said thermal-sprayed powder metal material.

12. A method according to Claim 5, wherein said body is a piston ring.

## Patentansprüche

1. Verfahren zum Bilden einer verschleißfesten Komponente, die folgenden Schritte umfassend: thermisches Spritzen eines Pulvermetallmaterials, wobei das Pulvermetallmaterial aus 3,0 bis 7,0 Gew.-% Kohlenstoff, 10,0 bis 25,0 Gew.-% Chrom, 1,0 bis 5,0 Gew.-% Wolfram, 3,5 bis 7,0 Gew.-% Vanadium, 1,0 bis 5,0 Gew.-% Molybdän, nicht mehr als 0,5 Gew.-% Sauerstoff besteht und der Rest Eisen und Verunreinigungen ist, auf Grundlage des Gesamtgewichts der Pulvermetallzusammensetzung.

2. Verfahren nach Anspruch 1, wobei der Schritt des thermischen Spritzens eine Technik des thermischen Spritzens ist, ausgewählt aus der Gruppe, bestehend aus: Pulverflammspritzen, Plasmaspritzen, Kaltspritzen und Hochgeschwindigkeitsflammspritzen (HVOF).

3. Verfahren nach Anspruch 1, wobei die Technik des thermischen Spritzens Folgendes beinhaltet: Bereitstellen einer Brennkammer, die ein Gemisch aus Kraftstoff und Sauerstoff enthält; Entzünden des Gemischs aus Kraftstoff und Sauerstoff; und Zuführen des Pulvermetallmaterials in die Brennkammer nach dem Schritt des Entzündens, um das Pulvermetallmaterial zu beschleunigen.

4. Verfahren nach Anspruch 3, wobei der Schritt des Entzündens Erzeugen eines Drucks in der Brennkammer und Beschleunigen des Pulvermetallmaterials bis zu einer Überschallgeschwindigkeit beinhaltet.

5. Verfahren nach Anspruch 1, beinhaltend Bereitstellen eines Körpers und wobei der Schritt des Spritzens Spritzen des Pulvermetallmaterials auf den Körper beinhaltet.

6. Verfahren nach Anspruch 1, wobei der Schritt des Spritzens die verschleißfeste Komponente bildet, und bei der verschleißfesten Komponente handelt es sich um einen Kolbenring, der eine Innenfläche, die eine Mittelachse umgibt, und eine Außenfläche, die gegenüber der Innenfläche liegt, darstellt.

7. Verfahren nach Anspruch 1, beinhaltend Bilden des Pulvermetallmaterials durch die folgenden Schritte:
Bereitstellen einer geschmolzenen auf Eisen basierenden Legierung, beinhaltend 3,0 bis 7,0 Gew.-% Kohlenstoff, 10,0 bis 25,0 Gew.-% Chrom, 1,0 bis 5,0 Gew.-% Wolfram, 3,5 bis 7,0 Gew.-% Vanadium, 1,0 bis 5,0 Gew.-% Molybdän, nicht mehr als 0,5 Gew.-% Sauerstoff und mindestens 40,0 Gew.-% Eisen auf Grundlage des Gesamtgewichts der geschmolzenen auf Eisen basierenden Legierung;
Zerstäuben der geschmolzenen auf Eisen basierenden Legierung, um zerstäubte Tröpfchen der auf Eisen basierenden Legierung bereitzustellen; und
Mahlen der zerstäubten Tröpfchen.

8. Verfahren nach Anspruch 7, wobei der Schritt des Zerstäubens Bilden von Metallcarbiden in der auf Eisen basierenden Legierung in einer Menge von mindestens 15,0 Vol.-% auf Grundlage des Gesamtvolumens der auf Eisen basierenden Legierung beinhaltet.

9. Verfahren nach Anspruch 8, wobei die Metallcarbide ausgewählt sind aus der Gruppe, bestehend aus: M8C7, M7C3, M6C, wobei M mindestens ein Metallatom ist und C Kohlenstoff ist.

10. Verfahren nach Anspruch 9, wobei M8C7 (V63Fe37)8C7 ist; M7C3 ausgewählt ist aus der Gruppe, bestehend aus: (Cr34Fe66)7C3, Cr3.5Fe3.5C3 und Cr4Fe3C3; und M6C ausgewählt ist aus der Gruppe, bestehend aus: Mo3Fe3C, Mo2Fe4C, W3Fe3C und W2Fe4C.

11. Verfahren nach Anspruch 1, wobei das Pulvermetallmaterial aus Folgendem besteht: 3,8 Gew.-% Kohlenstoff, 13,0 Gew.-% Chrom, 2,5 Gew.-% Wolfram, 6,0 Gew.-% Vanadium, 1,5 Gew.-% Molybdän, 0,2 Gew.-% Sauerstoff, Verunreinigungen in einer Menge von nicht mehr als 2,0 Gew.-% und wobei der Rest Eisen ist, auf Grundlage des Gesamtgewichts des thermisch gespritzten Pulvermetallmaterials.

12. Verfahren nach Anspruch 5, wobei der Körper ein Kolbenring ist.

## Revendications

1. Procédé de formation d'un composant résistant à l'usure, comprenant les étapes de :
pulvérisation thermique d'un matériau métallique en poudre, dans lequel le matériau métallique en poudre est constitué par 3,0 à 7,0 % en poids de carbone, 10,0 à 25,0 % en poids de chrome, 1,0 à 5,0 % en poids de tungstène, 3,5 à 7,0 % en poids de vanadium, 1,0 à 5,0 % en poids de molybdène, pas plus de 0,5 % en poids d'oxygène, et le reste étant du fer et des impuretés, sur la base du poids total de la composition métallique en poudre.

2. Procédé selon la revendication 1 dans lequel l'étape de pulvérisation thermique est une technique de pulvérisation thermique sélectionnée parmi le groupe constitué par : pulvérisation par flamme de poudre, pulvérisation au plasma, pulvérisation à froid, et pulvérisation d'oxy-combustible à haute vitesse (HVOF).

3. Procédé selon la revendication 1 dans lequel la technique de pulvérisation thermique inclut la fourniture d'une chambre de combustion contenant un mélange de combustible et d'oxygène ; l'allumage du mélange de combustible et d'oxygène ; et l'introduction du matériau métallique en poudre jusque dans la chambre de combustion après l'étape d'allumage pour accélérer le matériau métallique en poudre.

4. Procédé selon la revendication 3 dans lequel l'étape d'allumage inclut la création d'une pression dans la chambre de combustion, et l'accélération du matériau métallique en poudre jusqu'à une vitesse supersonique.

5. Procédé selon la revendication 1 incluant la fourniture d'un corps, et dans lequel l'étape de pulvérisation inclut la pulvérisation du matériau métallique en poudre sur le corps.

6. Procédé selon la revendication 1 dans lequel l'étape de pulvérisation forme le composant résistant à l'usure, et le composant résistant à l'usure est un segment de piston présentant une surface interne entourant un axe central et une surface externe faisant face à la surface interne.

7. Procédé selon la revendication 1 incluant la formation du matériau métallique en poudre par les étapes de :
fourniture d'un alliage à base de fer fondu incluant 3,0 à 7,0 % en poids de carbone, 10,0 à 25,0 % en poids de chrome, 1,0 à 5,0 % en poids de tungstène, 3,5 à 7,0 % en poids de vanadium, 1,0 à 5,0 % en poids de molybdène, pas plus de 0,5 % en poids d'oxygène, et au moins 40,0 % en poids de fer, sur la base du poids total de l'alliage à base de fer fondu ;
atomisation de l'alliage à base de fer fondu pour fournir des gouttelettes atomisées d'alliage à base de fer ; et
broyage des gouttelettes atomisées.

8. Procédé selon la revendication 7, dans lequel l'étape d'atomisation inclut la formation de carbures de métaux dans l'alliage à base de fer dans une quantité d'au moins 15,0 % en volume, sur la base du volume total de l'alliage à base de fer.

9. Procédé selon la revendication 8, dans lequel les carbures de métaux sont sélectionnés parmi le groupe constitué par : M8C7, M7C3, M6C, dans lequel M est au moins un atome de métal et C est du carbone.

10. Procédé selon la revendication 9, dans lequel M8C7 est (V63Fe37)8C7 ; M7C3 est sélectionné parmi le groupe constitué par : (Cr34Fe66)7C3, Cr3,5Fe3,5C3, et Cr4Fe3C3 ; et M6C est sélectionné parmi le groupe constitué par : Mo3Fe3C, Mo2Fe4C, W3Fe3C, et W2Fe4C.

11. Procédé selon la revendication 1, dans lequel le matériau métallique en poudre est constitué de : 3,8 % en poids de carbone, 13,0 % en poids de chrome, 2,5 % en poids de tungstène, 6,0 % en poids de vanadium, 1,5 % en poids de molybdène, 0,2 % en poids d'oxygène, des impuretés en une quantité de pas plus de 2,0 % en poids et le reste étant du fer, sur la base du poids total dudit matériau métallique en poudre pulvérisé par pulvérisation thermique.

12. Procédé selon la revendication 5, dans lequel ledit corps est un segment de piston.
